

# UNITED STATES PATENT OFFICE.

HUGH C. SICARD, OF BUFFALO, NEW YORK, ASSIGNOR TO UNITED STATES FERRO-  
ALLOYS CORPORATION, OF NEW YORK, N. Y., A CORPORATION OF NEW YORK.

## ALLOY OF IRON, CHROMIUM, AND TITANIUM AND PROCESS FOR THE PRODUCTION THEREOF.

1,346,343.

Specification of Letters Patent. Patented July 13, 1920.

No Drawing.

Application filed August 18, 1919. Serial No. 318,331.

*To all whom it may concern:*

Be it known that I, HUGH C. SICARD, a citizen of the United States of America, and a resident of the city of Buffalo, county of Erie, and State of New York, have invented a new and useful Alloy of Iron, Chromium, and Titanium and Processes for the Production Thereof, of which the following is a full, clear, and exact description.

10 This invention relates generally to the manufacture of chrome steel, that is, a steel containing various amounts of chromium. In the manufacture of chrome steel, it is well known that much difficulty is experienced in obtaining the desired quality 15 of product owing to the fact that some of the added chromium is oxidized by the oxids contained in the steel.

I have found that if an alloy of iron, 20 chromium and titanium, is used for making the chrome steel, the titanium, being more readily oxidized than the chromium, can be used to eliminate the oxids in the steel and thus protect the chromium from oxidation when it is added to the steel. This 25 invention is designed to overcome the difficulties of oxidation above referred to.

In making this alloy, I use as a source of 30 chromium, the chromium ore known as chromite which contains from 40% to 57% chromic oxid ( $Cr_2O_3$ ), from 10% to 20% of iron oxid ( $FeO$ ), and certain impurities such as alumina, magnesia, etc. As a source of titanium, I use a titaniferous ore, and 35 preferably rutile which contains 95% or more titanic oxid ( $TiO_2$ ).

The materials above named are mixed with scrap iron which supplies the iron content of the alloy and there is introduced 40 into the mixture an amount of carbon sufficient not only to reduce the chromic oxid and the titanic oxid, but an excess thereof so as to form, in the finished alloy, carbids of chromium, titanium and iron. When 45 necessary, such fluxes as sand, lime and the like may be added to the mixture in order to slag off the impurities contained therein.

The mixture is smelted in an open, electric furnace, for example, of the Siemens 50 type. Upon reduction, this mixture gives a bath of ferro-chromium, titanium and a slag. After reduction, they may be tapped separately or together as desired by the same tap-hole.

I have found this alloy to be a complex 55 carbid of chromium, titanium and iron, the amount of carbon varying from 3% to 9%. When added to molten steel the titanium content, on account of its great affinity for oxygen, will oxidize first, thus avoiding any 60 great loss of chromium.

One of the best alloys that I have found is one which contains the elements named in the following proportions:

|          |                 |    |
|----------|-----------------|----|
| Chromium | from 55% to 75% | 65 |
| Titanium | about 5%        |    |
| Carbon   | from 6% to 10%  |    |
| Iron     | from 34% to 10% |    |

It should be noted, however, that I have 70 been using alloys having titanium contents both lower and higher than above set forth. I have been able to secure very good results from a titanium content of from 1% to 16%. It is to be understood, therefore, that the 75 above percentages may be substantially varied and still the desirable results secured from the practice of my invention, that is, the results of protecting the chromium from being oxidized. It is, of course, 80 understood that there are usually unavoidably present in the finished products, some impurities such as silicon and aluminum.

Having thus described my invention, what 85 I claim is:

1. A method for the production of alloys 90 of iron, chromium and titanium comprising the mixture of chromium ore, rutile ore, scrap iron and carbon in sufficient quantity not only to reduce the chromium and titanium oxids present in the ores but enough to combine with the chromium, titanium and iron to form a complex carbid in the finished alloy, and then smelting this mixture in an electric furnace. 95

2. A method for the production of alloys 100 of iron, chromium and titanium comprising the mixture of a sufficient quantity of chromium ore to yield from 55% to 75% chromium in the finished product, a sufficient quantity of rutile ore to yield from 1% to 16% titanium in the finished product, carbon in such an excess quantity over that required for the reduction of the oxids that the finished product will contain from 105 6% to 10% carbon and a sufficient quantity of scrap iron so that the balance of percentage in the finished product will have an

iron content and then smelting this mixture in an electric furnace.

3. A method for the production of alloys of iron, chromium and titanium comprising the mixture of chromium ore, rutile ore, scrap iron and carbon in sufficient quantity not only to reduce the chromium and titanium oxids present in the ores but enough to combine with the chromium, titanium and iron to form a complex carbide in the finished alloy, a sufficient quantity

of a suitable flux to make a fusible slag, and then smelting this mixture in an electric furnace.

4. As a new article of manufacture an alloy of chromium, titanium and iron composed of from 55% to 75% chromium, from 1% to 16% titanium, from 6% to 10% carbon and the balance iron.

In testimony whereof I have hereunto signed my name.

HUGH C. SICARD.